

## UNITED STATES PATENT OFFICE.

HEINRICH WOHLWILL, OF HAMBURG, GERMANY, ASSIGNOR TO THE FIRM OF  
NORDDEUTSCHE AFFINERIE, OF HAMBURG, GERMANY.

## PROCESS OF REFINING GOLD.

961,924.

No Drawing.

Specification of Letters Patent. Patented June 21, 1910.

Application filed March 10, 1909. Serial No. 482,476.

*To all whom it may concern:*

Be it known that I, HEINRICH WOHLWILL, a subject of the Emperor of Germany, residing at 31-35 Elbstreet, Hamburg, German Empire, have invented new and useful Improvements in Processes of Refining Gold, of which the following is a specification.

This invention has reference to the purification of impure gold, or gold alloys, and 10 has particular reference to an electrolytic method of producing chemically pure gold from impure gold alloys, by employing the same as the anode in a suitable electrolytic bath.

15 The present invention constitutes an improvement on the processes described and claimed in Letters Patent, Nos. 625,863 and 625,864, granted to Emil Wohlwill, May 30, 1899.

20 In treating gold containing a relatively large percentage of silver as the anode in an electrolytic bath, consisting of a gold solution containing free hydrochloric acid or chlorids, according to the method described 25 in the patents above referred to, it has been found in practice, that when the proportion of silver in the material to be refined, exceeds six per cent., it is necessary, periodically, to mechanically remove the deposit of

30 chlorid of silver which forms upon, and covers the anode. If this removal of the chlorid of silver is omitted, gaseous chlorin is evolved at the anode, and interferes with the operation of the process. It has been

35 found that the greater the density of the current used, and the greater the percentage of silver in the gold anode, the sooner this condition obtains. For this reason, the process cannot be satisfactorily employed to

40 purify many varieties of gold coming from the mines, except by the use of a current of considerably lower density than can be employed in the purification of varieties of gold containing a smaller proportion of sil-

45 ver. By reason of the necessity of employing such current of lower current density, in refining gold containing a considerable percentage of silver, the operation is prolonged, and the removal of the chlorid of sil- 50 ver from the anode materially increases the cost of the process.

Now, I have found that it is possible to wholly prevent the development of chlorin

at the surface of the anode, and consequently to refine gold containing a very large percentage of silver by electrolysis in materially less time and at considerably lower expense than has been possible by the method hereinbefore referred to, by using an asymmetrical alternating electric current instead of a direct current.

55 Asymmetrical currents are produced either by commuting a direct current at small and unequal intervals of time, as for example, alternately every 1/50 and 3/50 seconds, or such currents may be produced by the simultaneous use of a direct current and an alternating current connected in parallel. I prefer however, to produce the asymmetrical current in a still different way, to 65 wit by connecting a source of direct current and a source of alternating current in series. This I commonly do by connecting a direct current dynamo and an alternating current dynamo in a series. It will be understood 70 that in an asymmetrical alternating current, the curve of the current will be equal to the curve of an ordinary alternating current, but it will oscillate, not on the zero value, but on the value of the direct current as the 75 zero line.

The quantitative effect of asymmetrical currents when applied to the refining of gold in accordance with the hereinbefore referred to process, is practically the same 85 as that of the direct current alone; that is to say, the quantity of gold, dissolved from the anode, and precipitated at the cathode, is practically equal to the quantity calculated from the strength of the direct current 90 alone, in accordance with Faraday's law. The advantageous effect of the alternating component of the asymmetrical current is however, exhibited in various ways. For example, as soon as the alternating current 95 is led into the direct current circuit, in which the electrolytic bath is included, the electric tension of the bath indicated on a direct current voltmeter falls, and the greater the strength of the alternating current, the greater the fall in the electric tension of the bath. Both poles exhibit a change in their manner of action, the change being especially noteworthy in respect of the anode.

100 By reason of the employment of the al-

ternating current with the direct current, the latter can be considerably increased without producing an evolution of chlorin at the anode, consequently the necessity of 5 removing deposits of chlorids from the anode is avoided.

When currents exceed a certain limit of density, in the present process, there is produced a slight evolution of oxygen, at the 10 anode. This evolution is however, so insignificant in volume, that the loss of current produced thereby, is without importance, and such evolution has in fact, a slightly 15 advantageous feature in that it facilitates the falling off of the deposit of chlorid of silver which forms upon the anode. When the current density is materially increased over the limit referred to, the development of oxygen becomes greater, and thereby the 20 loss of current becomes material.

It may be here stated, that the smaller the proportion of silver, and the higher the ratio of the alternating current to the strength of the direct current, the higher 25 will be the permissible density of the direct current. Therefore, in the use of the asymmetrical current, the development of any considerable amount of gas at the anode, as exhibited by the detachment of more than 30 single small bubbles from the anode, indicates that the strength of the direct current is too great, and the direct current must therefore, either be moderated or the strength of the alternating current increased. For example, impure gold containing 35 about ten per cent. of silver, according to the old process hereinbefore referred to, permits of no higher anodic density of the current than about 750 amperes to the 40 square meter, and necessitates the scraping off of deposits of silver chlorid from the anode every three-quarters of an hour. The same gold, can however, be treated in accordance with the present process with an 45 asymmetrical current, the alternating component of which has a strength of approximately 1 to 1.1 times that of the direct current, with a density of the direct current of 1250 amperes to the square meter, without 50 rendering any scraping off of the chlorid of silver from the anode necessary. The present process also renders possible, the treatment of gold alloys containing a considerably larger proportion of silver than 55 can be satisfactorily treated by the use of the direct current alone. For example, gold containing twenty per cent. of silver can be satisfactorily refined by the present process, by using an asymmetrical current, the 60 strength of the alternating component of which is to that of the strength of the direct current component as 1.7 is to 1, with a density of the direct current component of 1200 amperes to the square meter. With a

somewhat lower density of the direct current component, the process can be used for the refining of gold still richer in silver; in fact, the use of the asymmetrical current in accordance with the present process permits of the purification of all classes of 70 gold which are encountered in actual practice.

The use of asymmetrical alternating currents, and particularly the fact of being able to use direct currents of high density 75 therein, carries with it a still further advantage. In the electrolytic treatment of gold with a direct current of the density commonly used in gold solutions, containing an excessive quantity of hydrochloric acid 80 or chlorids, it is found that about ten per cent. of the quantity of gold, of the anodes, falls in minute particles into the slimes, from which it must be recovered by a separate chemical process. When, however, the 85 asymmetrical alternating current is used in the same situation, only a small amount of gold falls into the slimes and this only at the beginning of treatment, when the plate has not yet been covered with silver chlorid. 90 After this, practically no gold whatever, falls into the slimes, so that, in the operation of the present process, the slimes consist almost exclusively of chlorid of silver. In as much however as a small quantity of 95 gold falls into the slimes at the beginning of the treatment, and some gold particles arising from the mechanical disintegration of the anodes, fall into the slimes at the end of the treatment, the presence of gold in the 100 slimes cannot be wholly avoided; but this quantity rarely exceeds one per cent. of the quantity of the gold treated. Furthermore, if the use of currents of particularly high densities as for example, of a density in 105 excess of 1000 amperes to the square meter, is not of importance, the process offers the signal advantage that the quantity of hydrochloric acid or chlorids to be added to the electrolytic bath, may be materially less 110 than the quantity necessary when the direct current is used alone. By the use of asymmetrical alternating currents in accordance with the present process, gold can be refined with direct current densities of 1000 115 amperes or less to the square meter in a solution heated from 60 to 70° C., and containing only from about 1½ to 2 per cent. hydrochloric acid of 1.19 specific gravity, while in the treatment with direct currents, there is required about four times as much acid, that is to say about 7 per cent. hydrochloric acid. On the other hand, the heating of the bath to a temperature of about 60 or 70° C., can be dispensed with in the present process 120 when the proportion of hydrochloric acid in the solution amounts to 7 per cent. or more, providing the density of the direct 125

current component is not allowed to exceed from 600 to 1000 amperes to the square meter.

In the electrolytic treatment of gold in accordance with the old process hereinbefore referred to, the heating of the bath is absolutely essential, as the direct current when used alone, in the cold bath, even though below the requisite density of current, 500 amperes to the square meter, produces a precipitation of the gold in the form of a powder which varies in color from dark brown to black. The use of an asymmetrical current not only renders it possible to increase the cathodic density of the current as well as the anodic density of the current, in a warm solution, but also to refine the gold in a cold solution by the use of asymmetrical currents whose direct component has a density below 1000 amperes to the square meter, and obtain perfectly coherent precipitates.

In the practical operation of the process in its preferred embodiment, we proceed as follows: A direct current dynamo and an alternating current dynamo are connected in series in a circuit including the electrolytic bath and the direct current dynamo is excited until a polarized direct current ammeter inserted in the circuit, indicates the desired strength of the direct current. If this desired strength of the direct current is represented by  $i_d$ , and if it is desired to work with a virtual intensity of the alternating current represented by  $i_a$ , the virtual intensity of the total current obtained by the combined use of the two currents, can be calculated according to the formula

$$i_t = \sqrt{i_d^2 + i_a^2}$$

This total current can only be measured by a hot wire instrument. In addition to the direct current ammeter, a hot wire ammeter must therefore also be inserted in the asymmetrical current circuit. The alternating current dynamo is then excited until the hot wire ammeter indicated the desired current intensity  $i_t$ . For instance, if the strength of the direct current is to be equal to the strength of the alternating current, as for example, to 200 amperes, the hot wire ammeter must indicate

$$\sqrt{80000} = 283 \text{ amperes.}$$

The total voltage from which the power consumption is to be calculated, is indicated by a hot wire voltameter. The degree voltage depends of course, on the strength of the total current. For example, if gold is being treated, which contains about 10 per cent. of silver, a density of the direct current component of about 1250 amperes to the square meter, and a density of the alternating current component which is equal to, or

not more than 10 per cent. greater, is advisable; that is to say, a density of the total current corresponding to from

$$\sqrt{(1250)^2 + (1250)^2} = 1767 \text{ to}$$

$$\sqrt{1250^2 + 1375^2} = 1858$$

amperes to the square meter. In this case, the voltage of the direct current component is about from 1 to 1.1 volts per bath, and the total voltage per cell as indicated on a hot wire voltameter, is about 1.4 volts. From this, the voltage of the alternating current component can be calculated as follows:

$$i_a = \sqrt{(1.4)^2 - (1.1)^2} = .866 \text{ volts.}$$

In calculating the capacity of the dynamos, it will be desirable to consider 1.3 volts as the maximum voltage of the direct current, and 1 as the maximum voltage of the alternating current, per bath. As the dynamos are connected in series, the armatures of both dynamos must be wound for the highest occurring strength of the total current,  $i_t$ . The frequency of the alternating current can be varied within the usual limits.

The strengths and voltage of the currents employed may vary widely according to the character of the gold to be refined. If the gold contains less than 10 per cent silver, the density of the direct current component can be advantageously increased, or, if preferred, the strength of the alternating component relative to the direct current component can be diminished.

It is found in practice, that the ratio of the strength of the alternating current to that of the direct current cannot be advantageously diminished below a certain limit. For instance, if the strength of the alternating current becomes less than .707 of that of the direct current combined current will cease to be an alternating current and will become a mere undulatory direct current of periodically varying strength, in which case, the peculiar advantages of the combined current hereinbefore set forth, are lost.

In the practice of my process, I ordinarily work with a gold chlorid solution heated from 60 to 70° C., and containing at least 7 per cent. of free hydro-chloric acid. In cases where too much importance is not attached to rapidity of treatment and one can therefore be satisfied with a density of the direct current between 500 and 1000 amperes to the square meter, the treatment can take place either at the temperature indicated, the bath containing hydrochloric acid in the proportion of from  $1\frac{1}{2}$  to 2 per cent. of the solution, or the treatment can take place with a cold solution in which case 7 per cent. of hydrochloric acid gas is employed. Instead of using hydrochloric acid in the gold chlorid solution, I may substi-

tute either wholly or partially therefore chlorids such for example, as sodium chlorid.

In the preferred practice of my process, I 5 employ thinly rolled sheets of fine gold as cathodes and introduce gold into the electrolyte in the form of a gold chlorid solution in proportion as the gold content of the 10 bath is diminished; in the operation of the process. In refining gold which contains a 15 material percentage of lead, I may advantageously introduce sulfuric acid to the bath, preferably in a quantity approximately equivalent to that of the free hydrochloric acid present.

While I somewhat prefer to employ hydro-chloric acid in the gold bath it is to be understood that I may advantageously use a metal or other chlorid and that such 20 chlorid is the equivalent of hydro-chloric acid for use in my process.

I claim:

1. A process of electrolytically refining gold or gold alloys, which consists in elec-

trolyzing a solution of a gold salt by passing 25 an asymmetrical alternating current therethrough, with such gold or gold alloy as the anode.

2. A process of electrolytically refining gold or gold alloys, which consists in electrolyzing a solution containing gold chlorid 30 and another chlorid with an excess of the latter, by passing an asymmetrical alternating current therethrough with such gold or gold alloy as the anode.

3. A process of electrolytically refining gold or gold alloys, which consists in electrolyzing a solution of gold chlorid, containing hydrochloric acid, by passing an 35 asymmetrical alternating current therethrough with such gold or gold alloy as the anode.

In testimony whereof I have affixed my signature in presence of two witnesses.

HEINRICH WOHLWILL.

Witnesses:

ERNEST H. L. MUMMENHOFF,  
IDA CHR. HUFERMAN.